

# United States Patent Office

2,715,070

Patented Aug. 9, 1955

1

2,715,070

## RUTILE BOULE AND METHOD OF MAKING THE SAME

Charles H. Moore, Jr., Indianapolis, Ind., assignor to National Lead Company, New York, N. Y., a corporation of New Jersey

No Drawing. Application April 29, 1954,  
Serial No. 426,583

7 Claims. (Cl. 106—42)

The present invention relates to rutile single crystal boules modified with respect to color and certain other physical properties, and to methods for the production of such boules.

Rutile is one of the three known crystal modifications of titanium dioxide. When substantially pure, a massive single crystal of rutile has gem-like properties with a very light straw color and reflectance, refraction and brilliance greater than that of a diamond. The rutile single crystal is, however, not as hard as a diamond. By means of the present invention rutile single crystals may be produced which have a nearly water-white color and increased hardness and toughness, i. e. are less brittle or non-brittle. In addition, the present invention permits finishing the boule by reoxidation in considerably less time than is required for a pure rutile single crystal boule.

The principal object of the present invention is the preparation of rutile single crystal boules having nearly water-white color and a hardness greater than that of a pure rutile single crystal and increased toughness, i. e. are less brittle than pure rutile single crystals or non-brittle. Another object of the invention is a method for producing a finished, oxidized rutile single crystal boule in considerably less time than is required for the preparation of a finished oxidized pure rutile single crystal boule. These and other objects of the present invention will become apparent from the following description.

In its broadest aspect the present invention contemplates a rutile single crystal boule containing a small amount of an aluminum compound in solid solution and characterized by having a nearly water white color and a hardness and toughness greater than that of a pure rutile single crystal, prepared according to the method of the present invention by progressively fusing a mixture of finely-divided  $TiO_2$  containing a small amount of alumina in a flame carrying an excess of an oxidizing gas and thereafter oxidizing the boule so formed.

In this description of the present invention the word "boule" is used in its currently accepted meaning to denote a characteristic shape or form of an artificially prepared massive single crystal having a rounded end, or meniscus, a more or less rod-like body portion and a tapering end, giving an over-all appearance in profile of an almond, or carrot.

This application is a continuation-in-part of my co-pending application Serial No. 89,816 filed April 26, 1949, now abandoned.

The general method to which the present invention relates is that described in co-pending application Serial No. 54,562, filed October 14, 1948, now abandoned, for the preparation of pure rutile single crystal boules.

According to the preferred method of the present invention, there is employed as starting material a substantially pure  $TiO_2$  which is very fine, fairly uniform and possesses an open structure with units capable of being rapidly melted. A  $TiO_2$  having an ultimate unit particle size of approximately 0.1 micron has proved especially satisfactory. In general, material having an

2

average particle size above about 5 microns should be avoided because such particles do not satisfactorily fuse under the conditions of the invention. A preferred method for preparing a  $TiO_2$  starting material especially adapted for the production of rutile single crystal boules is described in co-pending application, Serial No. 54,578 filed October 14, 1948, issued as Patent No. 2,521,392, September 5, 1950, wherein a double salt, ammonium-titanium-sulphate is calcined so that all of the ammonia and sulfate are removed by volatilization.

According to the present invention the small amount of alumina may be mixed with the  $TiO_2$  starting material in any convenient manner, for instance, by dry mixing. A more uniform mixture and, therefore, a preferred mixture may be prepared by adding aluminum sulfate, as a powder, slurry or solution to the double salt, ammonium-titanium-sulphate prior to calcination.

The amount of alumina,  $Al_2O_3$ , to be added to the  $TiO_2$  starting material is very small and should not exceed about 0.1%, calculated as  $Al_2O_3$  based on the weight of the  $TiO_2$ . The boule will consist of  $TiO_2$  and  $Al_2O_3$ , said  $Al_2O_3$  present in amount from about 0.005% to about 0.1%. The preferred amount lies between about 0.005% and 0.05%. When the amount of alumina is increased substantially above about 0.1% resulting boules fracture badly and this is to be avoided. With higher amounts up to 2.0% and more it is not possible to obtain single crystal formation. With amounts of  $Al_2O_3$  of about 0.1% and below a complete solid solution of the  $Al_2O_3$  in the  $TiO_2$  is formed from which a high quality unfractured boule is produced. The rutile single crystal boule of this invention consisting of titanium dioxide and alumina may, and often will, contain small amounts of various substances which may enter as impurities in the raw materials. These substances may be present only in such amount that the rutile single crystal structure of the boule and its color are not substantially affected.

In progressively fusing the starting mixture of  $TiO_2$  and  $Al_2O_3$  there should be employed a flame which carries an excess of an oxidizing gas, preferably oxygen. Preferably the fusion is carried out at a temperature of from 1825° C. to 1900° C. according to the method described in application Serial No. 54,562, supra, in which the particles of the starting mixture are entrained in a stream of oxygen in a tube constituting the center of a burner consisting of three concentric tubes. In this burner hydrogen is introduced to the flame through the intermediate tube and additional oxygen in excess over the amount required to combine with the hydrogen is introduced through the outer tube. Preferably, the ratio of oxygen to hydrogen by volume should be about 1:1 and should not be less than about 8.5 parts of oxygen to 9.5 parts hydrogen by volume.

The flame temperature should be carefully controlled during the formation of the boule. It has been found that satisfactory results are obtained when the temperature is held between about 1825° C. and 1900° C. around the area where the boule is formed. Rutile melts at about 1820° C. and therefore it is necessary to operate so that the temperature at the top of the boule is somewhat above the melting point, e. g. 1825° C. If the temperature is in excess of 1900° C. an excessively large portion of the boule melts at the top and the molten material boils and runs over the sides of the boule.

The excess of oxygen in the flame is necessary because at elevated temperatures, titanium dioxide gives up oxygen and is converted to lower, or sub-oxides of titanium, e. g.  $Ti_2O_3$ . This loss of oxygen proceeds with considerable rapidity under conditions produced by an oxyhydrogen flame wherein the  $TiO_2$  is fused and the loss is accelerated when the flame is neutral or reducing. Under

## 3

such conditions the formation of lower, or sub-oxides of titanium, is so great that mixtures of small crystals of various oxides of titanium are produced rather than a single crystal boule.

Even when operating with an excess of oxygen the boule as produced has a generally deep blue-black color indicative of some deficiency in oxygen. Therefore, in the order to produce the nearly water-white boule of the present invention, the blue-black boule has to be re-oxidized.

The reoxidation of the boule is preferably carried out by heating the blue-black boule in an oxidizing atmosphere, for instance, air or oxygen. The temperature of the treatment should be within the range from about 650° C. to about 1500° C. It has been found that at temperatures to any extent below 650° C. oxygen will not be appreciably incorporated into the rutile single crystal. There is a decided loss in brilliance, lustre and fire when the treatment is carried out above 1500° C. and at that temperature the rate of oxygen incorporated into the rutile crystal is excessively rapid and difficult to control. Preferably the oxidation should be carried out at about 1100° C. to 1300° C. to properly anneal the boule. The heating should be continued until the boule obtains the maximum degree of lightness of color. This time will usually be about one quarter of that required to fully oxidize a pure rutile boule.

As produced, the alumina containing rutile boule has a more or less frosted outer surface. When split, the interior surfaces of the pieces are vitreous and shiny and nearly water-white. They may be cut and polished to form beautiful gems, more brilliant than diamonds and having a white color compared to the characteristic straw or light yellow color of pure rutile.

A rutile boule made according to this invention containing 0.01% alumina was tested for hardness using a Tukon tester as described in the Handbook of the American Society of Metals, 1948 edition, page 96. A Knoop indenter was employed carrying a load of 400 grams. The Knoop number indicating hardness, obtained on a boule of this invention compared to that obtained on a pure rutile boule is shown in the table below.

TABLE

## Knoop hardness

[400 g. load applied parallel to "C" axis.]

| Rutile Boule containing 0.01% alumina | Pure Rutile Boule                                                                            |
|---------------------------------------|----------------------------------------------------------------------------------------------|
| 1030                                  | 900—at 200 g. load calculated to 400 g. basis; (surface fracturing occurred at 400 g. load). |

As shown above the alumina containing boule gave a Knoop number of 1030 with a 400 g. load. The pure rutile boule splintered and cracked under a 400 gram load showing brittleness and lack of toughness compared to the alumina containing boule. The pure rutile boule tested under a 200 gram load showed a hardness of 900 calculated on the same basis as the 400 gram load used in testing the alumina containing boule. Therefore it is evident that the alumina containing boule is tough, non-brittle and shows an increased hardness compared to a pure rutile boule.

The foregoing description has been given for purposes of illustration, but the invention is not to be limited thereto and various modifications and variations within the scope of the appended claims may be employed.

I claim:

1. A rutile single crystal boule consisting of titanium dioxide and alumina, said alumina present in amount from 0.005% to 0.1% by weight.
2. A rutile single crystal boule consisting of titanium dioxide and alumina, said alumina present in amount from 0.005% to 0.05% by weight.

3. A method for producing a rutile single crystal boule which comprises forming an intimate mixture consisting of finely-divided titanium dioxide and from 0.005% to 0.1% alumina by weight, and fusing said mixture in an oxidizing atmosphere at a temperature of from 1825° C. to 1900° C. to form a single crystal boule.

4. A method for producing a substantially white single crystal boule which comprises forming an intimate mixture consisting of finely-divided titanium dioxide and from 0.005% to 0.1% alumina by weight, and fusing said mixture in an oxidizing atmosphere at a temperature of from 1825° C. to 1900° C. to form a single crystal boule and heating said boule in an oxidizing atmosphere at a temperature of 650° C. to 1500° C. until a substantially white color is obtained.

5. A substantially white rutile single crystal consisting of titanium dioxide and alumina, said alumina present in amount from 0.005% to 0.1% by weight.

6. A single crystal of synthetic rutile consisting of titania and between 0.03% and 0.1% of alumina.

7. A single crystal of synthetic rutile consisting of titania and between 0.005% and 0.1% of alumina.

45

No references cited.

50